

1

2,944,898

## SENSITIZATION OF PHOTOGRAPHIC EMULSIONS

Dorothy J. Beavers, Charles V. Wilson, and James L. Graham, Rochester, N.Y., assignors to Eastman Kodak Company, Rochester, N.Y., a corporation of New Jersey

No Drawing. Filed Nov. 27, 1957, Ser. No. 699,198

17 Claims. (Cl. 96—66)

This invention relates to the sensitization of photographic silver halide emulsions with certain quaternary ammonium salts e.g. pyridinium and quinolinium salts.

The sensitization of photographic emulsions with compounds containing quaternary nitrogen atoms has been known for many years as shown by the Carroll U.S. Patent 2,271,623 granted February 3, 1942. A representative quaternary salt sensitizing agent of that patent is the compound ethylene-bis-oxymethylpyridinium perchlorate.

We have discovered certain compounds containing quaternary nitrogen radicals which exhibit improved properties as sensitizing agents for silver halide emulsions. Emulsions containing the compounds of the invention are appreciably more stable than emulsions containing the mentioned quaternary compounds. Accordingly, upon the aging of emulsions containing the new sensitizing agents, less fog is developed and the emulsion speed is maintained. Also, photographic emulsions containing the new quaternary nitrogen compounds maintain their speed over a wider range of development conditions than do emulsions sensitized with previously known alkylene-bis-pyridinium salts such as decamethylene-1,10-bis-pyridinium perchlorate. Thus emulsions containing the latter compound as a sensitizing agent can be expected to lose an appreciable amount of speed when developed with a developing solution of high sulfite content of the order of 100 grams of anhydrous sodium sulfite per liter, whereas the emulsion speed is maintained in such developers when the emulsion is sensitized with the quaternary salts of the present invention.

When the emulsions are sensitized with the quaternary salts of the invention and are used in processes of color photography, that is, in multilayer color films adaptable to the reversal process of color photography, the first development step with the usual Metol-hydroquinone developer produces less fog than when the emulsions are sensitized with other quaternary salts such as that of the above Carroll invention.

It is interesting to note that Howe and Glassett British Patent 566,314 and Vanselow and James PSA Section B, 36-40 (1953) have shown that certain quaternary nitrogen salts such as n-dodecylpyridinium bromide, n-dodecyltriethyl ammonium bromide, etc. are not effective in increasing speed when development is carried out with a p-phenylenediamine as the developing agent such as used in color photography. In fact, it was shown by these workers that development with the p-phenylenediamine developing agent in the presence of the quaternary nitrogen salts retarded the development rate. The quaternary salts of the present invention when employed in the emulsions as sensitizing agents unexpectedly do not retard the development rate when development is carried out with a p-phenylenediamine type developing agent.

The quaternary salt sensitizing agents of the invention

2

are bis-quaternary salts having the following two general Formulas A and B:

(A)  $Q(RNHCOO)_{n-1}R'OOCN(HANHCOOR')(OCONHR)_{n-1}Q'$

wherein  $n$  represents the integers 1 or 2, and therefore includes tetra- and bis-urethanes of the general structures I and II, respectively.

(I)  $QRNHCOOR'OCONHANHCOOR'OCONHRQ'$

(II)  $QROCONHANHCOORQ$

(B)  $QRNHCOOA(OCONHR')_{n-1}Q'$

wherein  $n$  represents the integers 1 or 2, and therefore includes bis- and mono-urethanes of the general structures III and IV, respectively.

(III)  $QRNHCOOAOCNHR'Q'$

(IV)  $QRNHCOOAQ'$

and ureas of the general structure VI.

(VI)  $QRNCONANCONR'Q'$

In the above formulas Q and Q' represent the same or different organic radicals containing quaternary nitrogen atoms such as trialkyl ammonium salt radicals, and cyclammonium salt radicals e.g. pyridinium salt radicals or quinolinium salt radicals. R and R' represent the same or different radicals, which may be alkylene, such as

— $(CH_2)_n$ —, and including a carbon chain separated by other atoms such as O or S, e.g., — $(CH_2)_nO(CH_2)_n$ — or — $(CH_2)_n-S-(CH_2)_n'$ ,  $n$  and  $n'$  being integers of from about 1 to 10. The total chain length of R and R' must be such that the number of "atoms" in the linear chain joining Q to Q' does not exceed about 30. (The term "atoms" as used herein refers solely to the actual elements that compose the chain and not to any groups that these elements may carry. For example, — $(CH_2)_{10}$ — is considered to be a 10-atom chain, the hydrogen atoms being disregarded;

— $(CH_2)_5CONH(CH_2)_5$ —

is a 12-atom chain, the oxygen and hydrogen atoms being disregarded.) A compound of the above structure

wherein the chain contains 34 atoms has been found not to be useful as a sensitizing agent. Likewise compounds having less than about 14 atoms in the chain are not very useful sensitizing agents, the sensitizing activity of the compounds decreasing rapidly in compounds having less than about 14 or more than about 30 atoms in the linear chain connecting Q to Q'. In a preferred embodiment of the invention, therefore, the compounds contain from about 14 to about 30 atoms in the chain.

In Formulas I and II above group A represents a linear chain of one or more atoms of carbon which may or may not contain sulfur, oxygen or nitrogen as an intermediate linkage.

In the above formulas the number of atoms comprising group A is limited by the number of atoms in R and R' since as mentioned above the total number of atoms in the chain connecting Q to Q' must not exceed about 30. Thus in Formula II, A may contain as many as 22 atoms in a linear chain when R and R' are methylene groups. However, in such compounds where A represents an alkylene group, the linear chain of group A can contain only 2 to about 22 carbon atoms since it has not been possible to synthesize compounds in which A equals a — $CH_2$ — group because the diisocyanate OCN— $CH_2$ —NCO required in the synthesis is not available.



reaction occurred, the temperature rising to 135°. After the exotherm had subsided, the mixture was heated on the steam bath for an additional three hours. The urethane was crystallized from a large volume of methanol. The beautiful white crystals (22.3 g., 85 percent) melted at 85.0-86.5°.

In larger scale reactions, dry benzene may be used as the solvent for the isocyanate, and the chlorohydrin added slowly to this solution. Otherwise, the exothermic reaction cannot be controlled. The insoluble urethane was filtered from the benzene at the finish of the reaction.

An analytical sample was obtained from methanol as a white crystalline solid of melting point 86-87.5°.

*Anal.*—Calc. for  $C_{20}H_{38}N_2Cl_2O_4$ : C, 54.5; H, 8.6; N, 6.4; Cl, 16.1. Found: C, 54.5; H, 8.7; N, 6.6; Cl, 15.9.

9,16-diaza-7,18-dioxa-8,17-dioxotetraacosane-1,24-bis (pyridinium perchlorate)



A mixture of 50 ml. of dry pyridine and 10 g. (0.023 mole) of 9,16-diaza-7,18-dioxa-8,17-dioxotetraacosane-1,24-dichloride was refluxed for four hours. The excess pyridine was removed from the orange oil on the steam bath under vacuum. Ethanol was added and removed in the above manner to remove last traces of pyridine. The oily salt was redissolved in 25 ml. of ethanol and added to a solution of 6.3 g. (0.045 mole) of sodium perchlorate monohydrate in 25 ml. of acetone. The mixture was concentrated on the steam bath to about 30 ml., and the precipitated sodium chloride filtered off. The solution was slowly saturated with ether while cooling in a Dry Ice-acetone bath. The precipitated white granular solid was dissolved in a minimum of methanol, and acetone slowly added while chilling in a Dry Ice-acetone bath. The product was obtained as a crystalline white solid weighing 12.0 g. (73 percent) and melting at 63-65°.

The analytical sample was obtained from a methanol-acetone mixture and melted at 63-65°.

*Anal.*—Calc. for  $C_{30}H_{48}N_4Cl_2O_{12}$ : C, 49.5; H, 6.6; N, 7.7; Cl, 9.8. Found: C, 49.6; H, 6.8; N, 7.8; Cl, 10.7.

### COMPOUND VIII

3,18-diaza-5,16-dioxa-4,17-dioxoecosane-1,20-dichloride

A mixture of 10 g. (0.057 mole) of 1,10-decamethylene diol and 12.2 g. (0.116 mole) of  $\beta$ -chloroethyl isocyanate was cautiously heated on the steam bath. At 70° an exothermic reaction took place which was controlled by cooling with ice water. After the exotherm had subsided, the solid was heated at 130° for three hours to insure complete reaction. The solid was recrystallized from 200 ml. of methanol; 19.6 g. (89.5 percent), melting point 107.5-109.5°.

If this reaction is run on larger scale, an inert solvent such as benzene or toluene should be used as the violently exothermic reaction cannot be controlled without solvent. The desired product can then be filtered from the resulting slurry in pure form.

An analytical sample was obtained by recrystallization from methanol, melting point 106.5-108.5°.

*Anal.*—Calc. for  $C_{16}H_{30}N_2O_4Cl_2$ : C, 50.0; H, 7.8; N, 7.3; Cl, 18.5. Found: C, 49.6; H, 7.9; N, 7.3; Cl, 18.2.

3,18-diaza-5,16-dioxa-4,17-dioxoecosane-1,20-bis (pyridinium perchlorate)



Five grams (0.013 mole) of 3,18-diaza-5,16-dioxa-4,17-dioxoecosane-1,20-dichloride and 50 ml. of pyridine were vigorously refluxed for three hours. The excess pyridine was removed from the oil under vacuum on the steam bath, until no odor of pyridine remained. The oil was dissolved in 25 ml. of methanol and added to a solution of 4.0 g. (0.0286 mole) of sodium perchlorate in 50 ml. of acetone. The slurry was heated on the steam bath for 30 minutes, and the sodium chloride removed by filtration. The filtrate on chilling gave seven grams of a white solid, melting point 80-90°. The crude solid was recrystallized twice from alcohol-acetone, 5.3 g. (61 percent). It melted at 120-122.5° when placed on the hot stage at 70°.

*Anal.*—Calc. for  $C_{26}H_{40}N_4O_{12}Cl_2$ : C, 46.5; H, 6.0; N, 8.3; Cl, 10.6. Found: C, 46.1; H, 6.0; N, 8.3; Cl, 10.9.

### COMPOUND VII

3,10,17,24-tetraza-5,8,19,22-tetraoxa-4,9,18,23-tetraoxohexacosane-1,26-bispyridinium perchlorate



A mixture of 12 g. of 5,12-diaza-3,14-dioxa-4,13-dioxohexadecane-1,16-diol [prepared as described by Petersen, Ann., 562, 220 (1948)] and 9 g. of  $\beta$ -chloroethyl isocyanate was heated on the steam bath until a clear melt was obtained. The mixture was allowed to stand at 70° for 15 hours, though it had set to a solid in about one-half hour. The crude product was recrystallized from a large volume of methanol to yield 15 g. of 1,26-dichloro-3,10,17,24-tetraza-5,8,19,22-tetraoxa-4,9,18,23-tetraoxohexacosane of M.P. 159-161°.

*Anal.*—Calc. for  $C_{18}H_{32}O_8N_4Cl_2$ : C, 42.9; H, 6.4; N, 11.1; Cl, 14.1. Found: C, 43.5; H, 6.4; N, 10.7; Cl, 14.0.

A solution of 8.6 g. of the dichloro compound obtained in 30 ml. of pyridine was refluxed for 2 hours. An oil separated from the solution during the heating.

The excess pyridine was removed under reduced pressure and the residue dissolved in methanol. This solution was treated with a solution of 6 g. of sodium perchlorate in methanol. After warming for 15 minutes, the sodium chloride that separated was removed by filtration. The filtrate was concentrated to a small volume and the

quaternary salt precipitated as a gum by the addition of ether. The liquid was decanted from the gum and the latter was triturated with ether. The ether was decanted and the residue taken up in acetone. On chilling the solution a solid separated. The filtrate was diluted with

ether and chilled to give a second crop of solid. The total solid (7.5 g.) was recrystallized first from acetone and then from methanol-ether. In all cases of recrystallization the product first separated as a gum which set to a solid on chilling. Final yield, 5 g.

*Anal.*—Calc. for  $C_{28}H_{42}O_1N_6Cl_2$ : C, 42.8; H, 5.4; N, 10.7; Cl, 9.0. Found: C, 42.0; H, 5.2; N, 10.1; Cl, 10.5.

In a similar manner other symmetrical tetra-urethanes having the general Formula I above may be prepared using the appropriate alcohols and isocyanates. In preparing the unsymmetrical tetra-urethanes where R and R' are different the diol compound is first reacted with 1 mol of the appropriate haloalkyl isocyanate followed by reaction with 1 mol of a different haloalkyl isocyanate.

### COMPOUND IX

3-aza-5-oxa-4-oxopentadecane-1,15-dichloride



Decamethylene chlorohydrin (19.3 g., 0.10 mole) and 10.5 g. (0.10 mole) of 2-chloroethyl isocyanate were added together giving a mildly exothermic reaction. After the exotherm had subsided, the oil was heated on the steam bath for five hours. Upon cooling, a white crys-

talline mass weighing 29.5 g. (99 percent yield) and melting at 32-35° was obtained.

The analytical sample (M.P. 40.5-43.0°) was obtained from ether upon chilling in a Dry-Ice-acetone bath.

*Anal.*—Calc. for  $C_{13}H_{25}Cl_2NO_2$ : C, 52.3; H, 8.4; N, 4.7; Cl, 23.8. Found: C, 52.9; H, 8.5; N, 4.9; Cl, 24.0.

**3-aza-5-oxa-4-oxopentadecane-1,15-bis(pyridinium perchlorate)**



Twenty-five ml. of dry pyridine and 5.0 g. (0.017 mole) of 3-aza-5-oxo-oxapentadecane-1,15-dichloride were refluxed for three hours. Excess pyridine was removed on the steam bath under vacuum. The oil was then dissolved in methanol and this solvent removed under vacuum.

The resultant yellow oil was dissolved in 25 ml. of methanol and added to a solution of 5.5 g. of sodium perchlorate monohydrate in 25 ml. of acetone. The slurry was concentrated to one-half of the original volume and the inorganic salt filtered off. The solvent was removed from the oil, the oil dissolved in acetone, and the traces of inorganic salt removed by filtration. All attempts to obtain a crystalline product were unsuccessful. The product was isolated as a water-soluble yellow oil weighing 6.5 g. (76.5 percent yield).

**UREAS**

**COMPOUND XI**

**4,17-dioxo-3,5,16,18-tetrazaeicosane-1,20-dichloride**

$\beta$ -Chloroethyl isocyanate (10.6 g., 0.10 mole) was dissolved in 400 ml. of dry ether in a one-liter flask equipped with stirrer and condenser. With efficient stirring a solution of 8.6 g. (0.05 mole) decamethylenediamine in 200 ml. of dry benzene was slowly added. A dense white solid began precipitating immediately. After the complete addition of the diamine solution, the slurry was refluxed for two hours, then cooled and filtered. The white solid was washed with ether and air dried; yield, 11.9 g. (62 percent), melting point 158-162°.

An analytical sample of the urea was obtained from a large volume of methanol, melting point 162.5-165.5°.

*Anal.*—Calc. for  $C_{16}H_{32}N_4O_2Cl_2$ : C, 50.1; H, 8.4; N, 14.6; Cl, 18.5. Found: C, 50.6; H, 8.4; N, 14.6; Cl, 17.8.

**4,17-dioxo-3,5,16,18-tetrazaeicosane-1,20-bis (pyridinium perchlorate)**



A mixture of 50 ml. of dry pyridine, 20 ml. of absolute ethanol, and 5.7 g. (0.015 mole) of 4,17-dioxo-3,5,16,18-tetrazaeicosane-1,20-dichloride was heated to reflux for two hours. The solvents were removed on the steam bath under vacuum. The oil was slurried several times with ether and the ether decanted in order to remove traces of pyridine.

The pyridinium chloride was dissolved in 25 ml. of methanol, and a solution of 5.0 g. (0.036 mole) of sodium perchlorate monohydrate in 25 ml. of acetone added. The mixture was heated on the steam bath; immediately a dense solid consisting of bis-pyridinium perchlorate and sodium chloride separated. A large volume of ether was

added to the chilled slurry and the solid filtered off. The solid was dissolved in 225 ml. of hot aqueous methanol (1:2). Upon chilling, 5.8 g. of a cream-colored solid precipitated, melting point 182.5-186.0°. Concentration of the filtrate gave an additional 2.2 g. of product, melting point 180-185°. Total yield, 80 percent.

An analytical sample was prepared by recrystallization from a methanol-water solution, melting point 182-185°.

*Analysis.*—Calc. for  $C_{26}H_{42}N_6O_1Cl_2$ : C, 46.6; H, 6.3; N, 12.5; Cl, 10.6. Found: C, 46.6; H, 6.5; N, 12.8; Cl, 11.0.

The following examples illustrate the use of the bis-quaternary salts of the invention in photographic emulsions:

**Example 1**

A high-speed bromoiodide emulsion was prepared chemically sensitized with sulfur and gold compounds and optically sensitized with a cyanine dye. The amounts of the bis-quaternary nitrogen compound shown in Table I below were added to samples of the emulsion alone and together with an azaindene stabilizing agent. The emulsion samples were then coated, exposed on a sensitometer and developed for 5 minutes at 68° F. in the developer given below. The speed, gamma and fog values obtained by sensitometric evaluation of the developed samples are also shown in the table. The speed values shown are expressed as 100 (1-log E) where E is the exposure in meter candle seconds required to produce in the emulsion a density of 0.3 above fog.

|                          |       |      |
|--------------------------|-------|------|
| Water                    | cc    | 500  |
| Elon                     | grams | 2.5  |
| Sodium sulfite anhydrous | do    | 30.0 |
| Hydroquinone             | do    | 2.5  |
| Sodium metaperborate     | do    | 10.0 |
| Potassium bromide        | do    | 0.5  |

TABLE I

| Number | Feature                                                                                                         | Speed | $\gamma$ | Fog  |
|--------|-----------------------------------------------------------------------------------------------------------------|-------|----------|------|
| 137353 | Control                                                                                                         | 316   | 1.23     | 0.15 |
| 137356 | 5, 12-Diaza-3, 14-dioxa-4, 13-dioxohexadecane-1, 16-bis(trimethylammonium-p-toluenesulfonate) (II) 0.75 g./mol. | 321   | 1.24     | .18  |
| 137361 | 4-Hydroxy-6-methyl-1, 3, 3a, 7-tetraazaindene (XXX) 3.0 g./mol.                                                 | 325   | 1.13     | .15  |
| 137366 | (XXX) 3.0 g./mol.+(II) 0.75 g./mol.                                                                             | 328   | 1.24     | .15  |
| 137367 | (XXX) 3.0 g./mol.+(II) 2.25 g./mol.                                                                             | 335   | 1.14     | .16  |

50

**Example 2**

An emulsion was provided as in Example 1 and the additions shown in Table 2 were made to samples of the emulsion. Sensitometric evaluation made as described in Example 1 gave the results shown in the table.

TABLE 2

| Number | Feature                                                                                            | Speed | $\gamma$ | Fog  |
|--------|----------------------------------------------------------------------------------------------------|-------|----------|------|
| 140911 | Control                                                                                            | 318   | 1.29     | 0.20 |
| 140915 | 9, 16-Diaza-7, 18-dioxa-8, 17-dioxotetraacosane-1, 24-bis(pyridinium perchlorate) (V) 0.75 g./mol. | 340   | 1.27     | .26  |
| 140921 | 4-Hydroxy-6-methyl-1, 3, 3a, 7-tetraazaindene (XXX) 3.0 g./mol.                                    | 325   | 1.31     | .19  |
| 140929 | (XXX) 3.0 g./mol.+(V) 0.75 g./mol.                                                                 | 344   | 1.22     | .24  |
| 140930 | (XXX) 3.0 g./mol.+(V) 2.25 g./mol.                                                                 | 353   | 1.35     | .24  |

70

**Example 3**

An emulsion was provided as in Example 1 but with the addition to samples of the emulsion of the compounds shown in Table 3. Processing was carried out as in Example 1 for evaluating the emulsion sensitivity and other characteristics of the emulsion.

TABLE 3. *Example 4*

| Number | Feature                                                                                                                 | Speed | $\gamma$ | Fog  |
|--------|-------------------------------------------------------------------------------------------------------------------------|-------|----------|------|
| 151977 | Control                                                                                                                 | 308   | 1.30     | 0.17 |
| 151984 | 3, 10, 17, 24-Tetraza-5, 8, 19, 22-tetra-oxa-4, 9, 18, 23-tetraoxo-1, 26-bis(pyridinium perchlorate) (VII) 0.75 g./mol. | 322   | 1.38     | .16  |
| 152005 | 4-Hydroxy-6-methyl-1, 3, 3a, 7-tetrazaindene (XXX) 3.0 g./mol.                                                          | 317   | 1.35     | .14  |
| 152000 | (XXX) 3.0 g./mol+(VII) 0.75 g./mol.                                                                                     | 322   | 1.38     | .16  |
| 152001 | (XXX) 3.0 g./mol+(VII) 2.25 g./mol.                                                                                     | 323   | 1.32     | .15  |

*Example 4*

An emulsion was prepared and tested as shown in Example 1 using the bis-quaternary compound shown in Table 4. The data of this example shows that additional speed increase can be effected by using a combination of a bis-quaternary compound of the invention such as III and a polyethylene glycol XXXI, i.e., a polyethylene oxide of average molecular weight of 1500 (PEG 1500).

TABLE 4

| Number | Feature                                                                                                                | Speed | $\gamma$ | Fog  |
|--------|------------------------------------------------------------------------------------------------------------------------|-------|----------|------|
| 146237 | Control                                                                                                                | 317   | 1.30     | 0.17 |
| 146242 | 6, 13-Di-4, 15-dioxa-5, 14-dioxooctadecane-1, 18-bis( $\gamma$ -pyridinium metho-p-toluenesulfonate) (III) 0.3 g./mol. | 331   | 1.32     | .20  |
| 146245 | 4-Hydroxy-6-methyl-1, 3, 3a, 7-tetrazaindene (XXX) 3.0 g./mol.                                                         | 328   | 1.35     | .16  |
| 146258 | (XXX) 3.0 g./mol+(III) 0.3 g./mol.                                                                                     | 335   | 1.31     | .20  |
| 146259 | (XXX) 3.0 g./mol+(III) 0.75 g./mol.                                                                                    | 337   | 1.13     | .19  |
| 146263 | (XXX) 3.0 g./mol+PEG 1500 (XXXI) 0.75 g./mol.                                                                          | 346   | 1.06     | .18  |
| 146269 | (XXX) 3.0 g./mol+(XXXI) 0.75 g./mol+(III) 0.3 g./mol.                                                                  | 351   | 1.01     | .20  |

*Example 5*

An emulsion was prepared and tested as in Example

| Number | Feature                                                                                            | Fresh Tests |          |      | Incubation 1 wk. 120° F. |          |      | 3 Months 78° F. Keeping |          |      |
|--------|----------------------------------------------------------------------------------------------------|-------------|----------|------|--------------------------|----------|------|-------------------------|----------|------|
|        |                                                                                                    | CR Sp.      | $\gamma$ | Fog  | CR Sp.                   | $\gamma$ | Fog  | CR Sp.                  | $\gamma$ | Fog  |
|        |                                                                                                    |             |          |      |                          |          |      |                         |          |      |
| 147810 | Control                                                                                            | 342         | 1.12     | 0.15 | 343                      | 1.01     | 0.16 | 337                     | 1.05     | 0.16 |
| 147820 | Hexadecamethylene-1,16-bis(pyridinium perchlorate) 0.15 g/mol AgX                                  | 356         | 1.10     | .24  | 359                      | 1.10     | .22  | 333                     | 1.20     | .20  |
| 147821 | Hexadecamethylene-1,16-bis(pyridinium perchlorate) 0.3 g/mol AgX                                   | 356         | 1.24     | .30  | 359                      | 1.02     | .34  | 359                     | 1.23     | .26  |
| 147822 | Hexadecamethylene-1,16-bis(pyridinium perchlorate) 0.6 g/mol AgX                                   | 355         | 1.17     | .29  | 345                      | .90      | .48  | 356                     | 1.23     | .31  |
| 147848 | 9,16-Di-7,18-dioxa-8,17-dioxotetraacosane - 1,24 - bis(pyridinium perchlorate) (V) 0.45 g./mol AgX | 351         | 1.10     | .19  | 356                      | 1.17     | .17  | 350                     | 1.32     | .17  |
| 147849 | 9,16-Di-7,18-dioxa-8,17-dioxotetraacosane - 1,24 - bis(pyridinium perchlorate) (V) 0.75 g./mol AgX | 354         | 1.18     | .18  | 359                      | 1.10     | .18  | 334                     | 1.30     | .20  |
| 147850 | 9,16-Di-7,18-dioxa-8,17-dioxotetraacosane - 1,24 - bis(pyridinium perchlorate) (V) 1.2 g./mol AgX  | 355         | 1.29     | .19  | 361                      | 1.28     | .19  | 339                     | 1.42     | .17  |

1 using the "inverse" urethane VIII as shown in the following table.

TABLE 5

| Number | Feature                                                                                            | Speed | $\gamma$ | Fog  |
|--------|----------------------------------------------------------------------------------------------------|-------|----------|------|
| 149878 | Control                                                                                            | 305   | 1.22     | 0.10 |
| 149885 | 3, 18-Di-5, 16-dioxa-4, 17-dioxotetraacosane-1, 20-bis(pyridinium perchlorate) (VIII) 0.75 g./mol. | 327   | 1.26     | .12  |
| 149888 | 4-Hydroxy-6-methyl-1, 3, 3a, 7-tetrazaindene (XXX) 3.0 g./mol.                                     | 313   | 1.10     | .10  |
| 149907 | (XXX) 3.0 g./mol+(VIII) 0.75 g./mol.                                                               | 324   | 1.03     | .11  |
| 149908 | (XXX) 3.0 g./mol+(VIII) 2.25 g./mol.                                                               | 325   | 1.05     | .12  |
| 149911 | (XXX) 3.0 g./mol+PEG 1500 (XXXI) 0.75 g./mol.                                                      | 333   | 1.02     | .12  |
| 149912 | (XXX) 3.0 g./mol+(XXXI) 0.75 g./mol+(VIII) 0.75 g./mol.                                            | 337   | 1.17     | .14  |

*Example 6*

An emulsion was prepared and tested as in Example 1 using the bis-quaternary urea compound X.

TABLE 6

| Number | Feature                                                                             | Speed | $\gamma$ | Fog  |
|--------|-------------------------------------------------------------------------------------|-------|----------|------|
| 147490 | Control                                                                             | 315   | 1.17     | 0.17 |
| 147481 | Hexamethylenebis-[3-(2-ureidopyridinium metho-p-toluenesulfonate)] (X) 0.75 g./mol. | 315   | 1.15     | .15  |
| 147491 | 4-Hydroxy-6-methyl-1, 3, 3a, 7-tetrazaindene (XXX) 3.0 g./mol+(X) 0.3 g./mol.       | 321   | 1.25     | .17  |
| 147494 | (XXX) 3.0 g./mol+(X) 0.75 g./mol.                                                   | 322   | 1.09     | .17  |
| 147495 | (XXX) 3.0 g./mol+(X) 0.75 g./mol.                                                   | 325   | 1.06     | .15  |
| 147505 | (XXX) 3.0 g./mol+PEG 1500 (XXXI) 0.75 g./mol.                                       | 343   | 1.05     | .17  |
| 147508 | (XXX) 3.0 g./mol+(XXXI) 0.75 g./mol+(X) 0.75 g./mol.                                | 343   | 1.01     | .17  |

*Example 7*

A fast bromoiodide emulsion was chemically sensitized with sulfur and gold compounds and optically sensitized with a combination of cyanine dyes. In addition, 3.0 grams per mole of silver halide of 4-hydroxy-6-methyl-1,3,3a,7-tetrazaindene and 0.75 gram per mole of silver halide of a polyethylene oxide of average molecular weight 1500 were added. The amounts of the compounds shown in Table 7 were then added and the emulsions coated. Testing was carried out as in Example 1 upon the freshly coated emulsion samples and other samples of each emulsion were incubated for 1 week at 120° F. and 50 percent relative humidity. Still other samples of each emulsion were stored under room conditions "78° F. Keeping" and developed with the same developing solution given in Example 1 with the result shown in Table 7. Consideration of the "fog" data in the table shows that the emulsions containing the compound V of the invention were more stable than the emulsions containing the alkylene bis-pyridinium compound of the prior art.

TABLE 7

| Number | Feature                                                                                            | Fresh Tests |          |      | Incubation 1 wk. 120° F. |          |      | 3 Months 78° F. Keeping |          |      |
|--------|----------------------------------------------------------------------------------------------------|-------------|----------|------|--------------------------|----------|------|-------------------------|----------|------|
|        |                                                                                                    | CR Sp.      | $\gamma$ | Fog  | CR Sp.                   | $\gamma$ | Fog  | CR Sp.                  | $\gamma$ | Fog  |
|        |                                                                                                    |             |          |      |                          |          |      |                         |          |      |
| 147810 | Control                                                                                            | 342         | 1.12     | 0.15 | 343                      | 1.01     | 0.16 | 337                     | 1.05     | 0.16 |
| 147820 | Hexadecamethylene-1,16-bis(pyridinium perchlorate) 0.15 g/mol AgX                                  | 356         | 1.10     | .24  | 359                      | 1.10     | .22  | 333                     | 1.20     | .20  |
| 147821 | Hexadecamethylene-1,16-bis(pyridinium perchlorate) 0.3 g/mol AgX                                   | 356         | 1.24     | .30  | 359                      | 1.02     | .34  | 359                     | 1.23     | .26  |
| 147822 | Hexadecamethylene-1,16-bis(pyridinium perchlorate) 0.6 g/mol AgX                                   | 355         | 1.17     | .29  | 345                      | .90      | .48  | 356                     | 1.23     | .31  |
| 147848 | 9,16-Di-7,18-dioxa-8,17-dioxotetraacosane - 1,24 - bis(pyridinium perchlorate) (V) 0.45 g./mol AgX | 351         | 1.10     | .19  | 356                      | 1.17     | .17  | 350                     | 1.32     | .17  |
| 147849 | 9,16-Di-7,18-dioxa-8,17-dioxotetraacosane - 1,24 - bis(pyridinium perchlorate) (V) 0.75 g./mol AgX | 354         | 1.18     | .18  | 359                      | 1.10     | .18  | 334                     | 1.30     | .20  |
| 147850 | 9,16-Di-7,18-dioxa-8,17-dioxotetraacosane - 1,24 - bis(pyridinium perchlorate) (V) 1.2 g./mol AgX  | 355         | 1.29     | .19  | 361                      | 1.28     | .19  | 339                     | 1.42     | .17  |

*Example 8*

The use of the bis-quaternary salts of the invention in color photography is illustrated in this example.

A sulfur and gold sensitized gelatino silver bromoiodide emulsion was ripened to maximum sensitivity. To this emulsion was added an optical sensitizing dye that extended the light sensitivity to 6000-7000 A. and a hydrophobic cyan color former suitably dispersed in a high boiling organic solvent. A portion of this liquid emulsion received no further treatment; to another portion was added one of the compounds described below. Both portions were coated on film support, and the dry films were exposed to red light in an intensity scale sensitometer. The exposed films were processed in the reversal Color Process 1 and the 5248 negative Color Process 2 with the

results shown in the following table. The Color Process 2 was carried out as described by Hanson and Kisner JSMPT 61 667-701 (1953) for the Color Negative Film, Type 5248, involving the steps of color development, fixation, silver bleaching and final fixation. Color Process 1 was carried out at 75° F. as follows:

|                             | Minutes |
|-----------------------------|---------|
| (1) Negative development    | 10      |
| (2) Reversal flash exposure | —       |
| (3) Color development       | 15      |
| (4) Silver bleaching        | 8       |
| (5) Fixing                  | 3       |

The negative developer had the following composition:

|                                              |       |      |
|----------------------------------------------|-------|------|
| Water, 90° F. (32 C.)                        | liter | 1.0  |
| Sodium hexametaphosphate                     | grams | 2.0  |
| N-methyl p-aminophenol sulfate               | do    | 6.0  |
| Sodium sulfite, desiccated                   | do    | 50.0 |
| Hydroquinone                                 | do    | 6.0  |
| Sodium carbonate, monohydrated               | do    | 35.0 |
| Potassium bromide                            | do    | 2.0  |
| Sodium thiocyanate                           | do    | 1.5  |
| 0.5% solution (6-nitrobenzimidazole nitrate) | cc    | 12.0 |
| 0.1% solution of potassium iodide            | cc    | 10.0 |

The color developing solution above had the following composition:

|                                                                                     |       |       |
|-------------------------------------------------------------------------------------|-------|-------|
| Water, 70 to 80 F. (21 to 27 C.)                                                    | liter | 1.0   |
| Benzyl alcohol                                                                      | cc    | 6.0   |
| Sodium hexametaphosphate                                                            | grams | 2.0   |
| Sodium sulfite, desiccated                                                          | do    | 5.0   |
| Trisodium phosphate                                                                 | do    | 40.0  |
| Potassium bromide                                                                   | gram  | 0.25  |
| 0.1% solution of potassium iodide                                                   | cc    | 10.0  |
| Sodium hydroxide                                                                    | grams | 6.5   |
| (4-amino-N-ethyl-N-β-methane sulfonamidoethyl)m-toluidine sesquisulfate monohydrate | grams | 11.33 |
| Ethylenediamine sulfate                                                             | do    | 7.8   |
| Citrazinic acid (2,6-dihydroxyisonicotinic acid)                                    | grams | 1.5   |

The silver bleaching solution above had the following composition:

|                        |       |      |
|------------------------|-------|------|
| Water 90 F. (32 C.)    | liter | 1.0  |
| Potassium dichromate   | grams | 5.0  |
| Potassium ferricyanide | do    | 70.0 |
| Potassium bromide      | do    | 20.0 |

The fixing baths above had the following composition:

|                      |       |       |
|----------------------|-------|-------|
| Water, 80 F. (27 C.) | liter | 1.0   |
| Sodium thiosulfate   | grams | 150.0 |
| Sodium bisulfite     | do    | 20.0  |

TABLE 8

| Number | Feature                           | Color Process 1<br>(Reversal)<br>Speed Increase<br>( $\Delta \log E$ ) <sup>1</sup> | Color Process 2<br>(5248 Negative)<br>Speed Increase<br>( $\Delta \log E$ ) <sup>2</sup> |
|--------|-----------------------------------|-------------------------------------------------------------------------------------|------------------------------------------------------------------------------------------|
| 19360  | Control                           |                                                                                     |                                                                                          |
| 19365  | Compound I, 2.0 g./mole<br>Ag X.  | +0.16                                                                               | +0.15                                                                                    |
| 19540  | Control                           |                                                                                     |                                                                                          |
| 19549  | Compound VI, 2.0 g./mole<br>Ag X. | +0.18                                                                               | +0.18                                                                                    |

<sup>1</sup> Determined by measuring the shift of the reversal dye curve on the Log E axis at a given density below maximum density.

<sup>2</sup> Determined by measuring the shift of the negative dye curve on the Log E axis at a given density above minimum density.

The bis-quaternary salts described above can be used in emulsions in the manner of the above examples in concentrations of the order of about 0.02 to 4 grams per mol of silver halide.

The emulsions may also be developed in the presence of the bis-quaternary salts by incorporating the salts into a developer solution. For example, when compound VI was added to the color developer (2 g. per liter) of Color

Process 2 of Example 8 and a multilayer color film having couplers in the emulsion layers was developed therein, speed increase was obtained particularly for the red and green sensitive emulsion layers.

As indicated in the above examples, it may be desirable to incorporate a stabilizing agent into the emulsion sensitized with the bis-quaternary salts of the invention to reduce fog to normal levels. Azaindenes particularly suitable for this purpose are those described in the Carroll et al. U.S. patent application Serial Nos. 627,135 and 627,136, filed December 10, 1956, for example, the following: 5-carboxy-4-hydroxy-1,3,3a,7-tetraazaindene, 1,2-bis(4-hydroxy-6-methyl-1,3,3a,7-tetraazaindene-5-yl)ethane, 1,2,3,4-tetrakis(4-hydroxy-6-methyl-1,3,3a,7-tetraazaindene-2-yl)butane, 2-amino-5-carboxy-4-hydroxy-1,3,3a,7-tetraazaindene, 4-hydroxy-2-β-hydroxy-ethyl-6-methyl-1,3,3a,7-tetraazaindene, 5-carboxy-4-hydroxy-1,3,3a,7-tetraazaindene, 7-hydroxy-1,2,3,4,6-pentazaindene, 2,4-dihydroxy-6-methyl-1,3,3a,7-tetraazaindene, 4-hydroxy-2-γ-hydroxypropyl-6-methyl-1,3,3a,7-tetraazaindene and 4-hydroxy-2(4-pyridyl)-6-methyl-1,3,3a,7-tetraazaindene.

The preparation of silver halide emulsions involves three separate operations: (1) the emulsification and digestion or ripening of the silver halide, (2) the freeing of the emulsion from aqueous soluble salts usually by washing, (3) the second digestion or after-ripening to obtain increased sensitivity (Mees, The Theory of the Photographic Process, 1942, page 3). The sensitizing agents may be added at any stage, preferably after the final digestion.

The photographic emulsions which we use are of the developing-out type and best results have been obtained with gelatino-silver bromoiodide emulsions. However, emulsions of varying silver halide content may be used.

The emulsions are chemically sensitized by any of the accepted procedures in addition to sensitizing with the bis-quaternary salts of the invention. The emulsions may be digested with naturally active gelatin, or sulfur compounds may be added such as those described in Sheppard U.S. Patents 1,574,944 and 1,623,499, and Sheppard and Brigham U.S. Patent 2,410,689.

The emulsions may also be treated with salts of the noble metals such as ruthenium, rhodium, palladium, iridium and platinum, all of which belong to group VIII of the periodic table of elements and have an atomic weight greater than 100. Representative compounds are ammonium chloropalladate, potassium chloroplatinate and sodium chloropalladate, which are used for sensitizing in amounts below that which produces any substantial fog inhibition, as described in Smith and Trivelli U.S. Patent 2,448,060, and as anti-foggants in higher amounts, as described in Trivelli and Smith U.S. Patents 2,566,245 and 2,566,263.

The emulsions may also be chemically sensitized with gold salts as described in Waller and Dodd U.S. Patent 2,399,083 or stabilized with gold salts as described in Damschroder U.S. Patent 2,597,856 and Yutzy and Leermakers U.S. Patent 2,597,915. Suitable compounds are potassium chloroaurite, potassium aurithiocyanate, potassium chloroaurate, auric trichloride and 2-aurosulfobenzothiazole methochloride.

The emulsions may also be chemically sensitized with reducing agents such as stannous salts (Carroll U.S. Patent 2,487,850), polyamines such as diethylene triamine Lowe and Jones U.S. Patent 2,518,698, polyamines such as spermine (Lowe and Allen U.S. Patent 2,521,925), or bis-(β-aminoethyl) sulfide and its water-soluble salts (Lowe and Jones U.S. Patent 2,521,926).

The emulsions may also contain polyalkylene oxides and derivatives thereof such as the polyethylene glycols, in addition to the bis-quaternary compounds of the invention. Suitable polyalkylene oxides and polyalkylene oxide derivatives are described in Blake U.S. Patent 2,441,389, May 11, 1948, Blake et al. U.S. Patents 2,400-

532, May 21, 1946, 2,423,549, July 8, 1947, and Jennings et al. U.S. Patent 2,577,127, December 4, 1951.

Other compounds useful for suppressing the fog level of the emulsion sensitized with the bis-quaternary compounds of the invention include the mercury compounds of Allen et al. U.S. Patent 2,728,663, Carroll and Murray U.S. Patent 2,728,664 and Leubner and Murray U.S. Patent 2,728,665, granted December 27, 1955, and the organic salts of U.S. patent application Serial No. 493,-2,784,090, granted March 5, 1957.

Other stabilizing agents may be added to the emulsions containing the bis-quaternary salts such as the metal inorganic salts of U.S. Patent application Serial No. 493,047, filed March 8, 1955 by J. E. Jones.

The chemical sensitizing agents and other addenda which we have described may be used in various kinds of photographic emulsions, e.g., various silver salts may be used as the sensitive salt such as silver bromide, silver iodide, silver chloride or mixed silver halides such as silver chlorobromide or silver bromoiodide.

The dispersing agent for the silver halide may be gelatin or other hydrophilic material such as collodion, albumin, cellulose derivatives or synthetic resins.

Since the coupler-containing emulsions sensitized as described with the bis-quaternary salts are adapted particularly for use in color photography, they will ordinarily comprise the emulsion layers of multilayer color films which emulsion layers are customarily differentially sensitized to the primary regions of the visible spectrum and contain coupler compounds producing dye images of colors complementary to the sensitivity of the emulsion layers. In a representative color film, one or more of the differentially sensitized emulsion layers may be sensitized with the bis-quaternary salts, and in a typical example emulsions sensitized to the red, green and blue regions of the spectrum are super-imposed on the support in that order and contain cyan, magenta and yellow color-forming coupler compounds respectively. A yellow filter layer such as yellow colloidal silver is advantageously interposed between the blue and green-sensitive emulsion layers.

Since the emulsion layers sensitized with the bis-quaternary salts of the invention may contain coupler compounds they can be readily processed by well known methods to yield color negatives directly or positive images by means of well known reversal processes. That is, after initial exposure of the emulsion to a subject a developer of the p-phenylenediamine type will produce a colored image negative in respect to the subject. Likewise, if development of the emulsion layer is first carried out with a non-color-forming developer followed by reversal exposure of the residual silver halide and then color development, a colored positive is obtained as described in the examples above.

The coupler compounds used in the emulsion layers sensitized with the ionic polyalkylene oxide derivatives, are any of the well known compounds which combine with the oxidation product of primary aromatic amino (p-phenylenediamines) silver halide color developing agents to form dyes, for example, the phenolic couplers of U.S. Patents 2,266,452, 2,362,598, 2,589,004, 2,474,293, 2,521,908, 2,423,730 and Fierke U.S. patent application 476,561; the pyrazolone couplers of U.S. Patents 1,969,479, 2,369,489, 2,600,788, 2,618,641, 2,511,231 and the open chain reactive methylene couplers of U.S. Patents 2,298,443, 2,652,329, 2,407,210, 2,271,238 and McCrosen et al. U.S. patent application Serial No. 575,099, filed March 30, 1956. Likewise, the emulsions may contain colored color-forming couplers as described in U.S. Patents 2,521,908, 2,706,684, 2,455,169, 2,694,703, 2,455,170 and 2,453,661.

ing groups such as  $\text{SO}_3\text{H}$  groups which render the couplers soluble in alkaline solution, the oily coupler solvent may be dispensed with and the couplers can be added to the emulsion from aqueous solutions as their alkali metal salts.

What we claim and desired to secure by Letters Patent of the United States is:

1. A photographic silver halide emulsion containing a quaternary ammonium salt having a general formula of  
10 the class consisting of



and



wherein Q and Q' each represent radicals of the class consisting of



- 25 wherein  $R^3$ ,  $R^4$  and  $R^5$  represent lower alkyl groups,  $Z$  represents the atoms necessary to complete a heterocyclic nucleus of the class consisting of pyridinium and quinolinium,  $R$  and  $R'$  each represent alkylene groups linked to the quaternary nitrogen atoms of said radicals,  $R^2$  represents a member of the class consisting of a hydrogen atom and an alkyl group of from 1 to 4 carbon atoms,  $n$  represents a positive integer of from 1 to 2,  $A$  represents a member of the class consisting of



and



- 50 wherein  $n'$  and  $n''$  represent positive integers of from about 1 to 10, there being from about 14 to about 30 atoms present in the shortest linear chain of atoms linking said quaternary nitrogen atoms.

- 55 2. A photographic silver halide emulsion containing a quaternary ammonium salt having the general formula

QRNHCOOR'OO CNHANHCOOR'OCNHRQ'

wherein Q and Q' represent radicals of the class consisting of



- 65 wherein  $R^2$ ,  $R^3$  and  $R^4$  represent lower alkyl groups,  $Z$  represents the atoms necessary to complete a heterocyclic nucleus of the class consisting of pyridinium and quinolinium,  $R$ ,  $R'$  and  $A$  each represent alkylene groups, there being from about 14 to about 30 atoms present in  
70 the shortest linear chain of atoms linking the quaternary nitrogen atoms of said radicals.

3. A photographic silver halide emulsion containing a quaternary ammonium salt having the general formula



wherein Q and Q' represent radicals of the class consisting of



wherein R<sup>2</sup>, R<sup>3</sup> and R<sup>4</sup> represent lower alkyl groups, Z represents the atoms necessary to complete a heterocyclic nucleus of the class consisting of pyridinium and quinolinium, R, R' and A each represent alkylene groups, there being from about 14 to about 30 atoms present in the shortest linear chain of atoms linking the quaternary nitrogen atoms of said radicals.

4. A photographic silver halide emulsion containing a quaternary ammonium salt having the general formula



wherein Q and Q' each represent radicals of the class consisting of



wherein R<sup>1</sup>, R<sup>2</sup> and R<sup>3</sup> represent lower alkyl groups, Z represents the atoms necessary to complete a heterocyclic nucleus of the class consisting of pyridinium and quinolinium, R and A each represent alkylene groups, there being from about 14 to about 30 atoms present in the shortest linear chain of atoms linking the quaternary nitrogen atoms of said radicals.

5. A method of increasing the speed of a silver halide emulsion layer which comprises developing said emulsion in the presence of a quaternary ammonium salt having a formula of the class consisting of



and



wherein Q and Q' each represent radicals of the class consisting of



wherein R<sup>3</sup>, R<sup>4</sup> and R<sup>5</sup> represent lower alkyl groups, Z represents the atoms necessary to complete a heterocyclic nucleus of the class consisting of pyridinium and quinolinium, R and R' each represent alkylene groups linked to the quaternary nitrogen atoms of said radicals, R<sup>2</sup> represents a member of the class consisting of a hydrogen atom and an alkyl group of from 1 to 4 carbon atoms, n represents a positive integer of from 1 to 2, A represents a member of the class consisting of



and



5

wherein n' and n'' represent positive integers of from about 1 to 10, there being from about 14 to about 30 atoms present in the shortest linear chain of atoms linking said quaternary nitrogen atoms.

6. A photographic silver halide emulsion containing the compound 5,12-diaza-3,14-dioxa-4,13-dioxo-hexadecane-1,16-bis(trimethylammonium p-toluene sulfonate).

7. A photographic silver halide emulsion containing the compound 6,13-diaza-4,15-dioxa-5,14-dioxa-octadecane-1,18-bis(N-methylpyridinium p-toluene sulfonate).

8. A photographic silver halide emulsion containing the compound 9,16-diaza-7,18-dioxa-8,17-dioxotetracosane-1,24-bis(pyridinium perchlorate).

9. A photographic silver halide emulsion containing the compound 3,10,17,24-tetraza-5,8,19,22-tetraoxa-4,9,18,23-tetroxohexacosane-1,26-bis(pyridinium perchlorate).

10. A photographic silver halide emulsion containing the compound 3,18-diaza-5,16-dioxa-4,17-dioxoeicosane-1,20-bis(pyridinium perchlorate).

11. The emulsion of claim 2 further containing a coupler compound reactive with the oxidation products of a phenylenediamine silver halide developing agent to form a dye.

12. The emulsion of claim 3 further containing a coupler compound reactive with the oxidation products of a phenylenediamine silver halide developing agent to form a dye.

13. The emulsion of claim 4 further containing a coupler compound reactive with the oxidation products of a phenylenediamine silver halide developing agent to form a dye.

14. The emulsion of claim 2 further containing an azaindene stabilizing agent.

15. The emulsion of claim 3 further containing an azaindene stabilizing agent.

16. The emulsion of claim 4 further containing an azaindene stabilizing agent.

17. The emulsion of claim 1 wherein the silver halide is sulfur and gold sensitized.

#### References Cited in the file of this patent

#### UNITED STATES PATENTS

- |    |           |                       |               |
|----|-----------|-----------------------|---------------|
| 50 | 2,288,226 | Carroll et al. -----  | June 30, 1942 |
|    | 2,419,975 | Trivelli et al. ----- | May 6, 1947   |
|    | 2,784,090 | Carroll -----         | Mar. 5, 1957  |

#### FOREIGN PATENTS

- |    |         |                 |               |
|----|---------|-----------------|---------------|
| 55 | 115,971 | Australia ----- | Oct. 15, 1942 |
|----|---------|-----------------|---------------|

UNITED STATES PATENT OFFICE  
CERTIFICATE OF CORRECTION

Patent No. 2,944,898

July 12, 1960

Dorothy J. Beavers et al.

It is hereby certified that error appears in the printed specification of the above numbered patent requiring correction and that the said Letters Patent should read as corrected below.

Column 13, line 9, strike out "salts of U.S. patent application Serial No. 493,—" and insert instead -- mercury compounds of Carroll et al U.S. patent --.

Signed and sealed this 4th day of April 1961.

(SEAL)

Attest: ERNEST W. SWIDER

XXXXXXXXXX

Attesting Officer

ARTHUR W. CROCKER  
Acting Commissioner of Patents